

## [54] SUPERCONDUCTING MATERIALS

- [75] Inventors: **Ushio Kawabe; Mitsuhiro Kudo; Shigeo Fukase; Masato Ishibashi**, all of Tokyo, Japan
- [73] Assignee: **Hitachi, Ltd., Japan**
- [22] Filed: **Dec. 1, 1972**
- [21] Appl. No.: **311,148**

## [30] Foreign Application Priority Data

Dec. 1, 1971 Japan..... 46-96271

- [52] U.S. Cl. .... **75/174; 148/32; 148/32.5; 148/133; 335/216**
- [51] Int. Cl. .... **C22c 27/00; H01f 1/04**
- [58] Field of Search ..... 335/216; 75/174; 148/32; 148/32.5, 133

## [56] References Cited

## UNITED STATES PATENTS

- |           |         |                 |          |
|-----------|---------|-----------------|----------|
| 3,244,490 | 4/1966  | Saur.....       | 75/174 X |
| 3,290,186 | 12/1966 | Rosi et al..... | 75/174 X |
| 3,544,316 | 12/1970 | Sahm et al..... | 75/174   |

## OTHER PUBLICATIONS

- Physical Review Vol. 152, No. 1, Dec. 2, 1966 pgs. 341-344.
- Z. Metallkde, Bd59 (1968) No. 9, Hunt & Ramm, pgs. 701-707.
- Metallurgy of Advanced Electronic Materials, Vol. 19, (1962) Gordon and Breach Science Pub. N.Y. pgs. 71-86.

Primary Examiner—C. Lovell  
Attorney, Agent, or Firm—Craig & Antonelli

## [57] ABSTRACT

A  $Nb_KAl$  type intermetallic compound superconducting material, in which part of Al is replaced with an element selected from a group consisting of Pb, Bi, Tl, Cu, Sb, Te, Y, Ce, Pr, Eu, Ca and Zn and, if necessary, part of Nb is replaced with Ta, is disclosed. This material has a critical temperature of 18°K or higher and a  $\beta$ -W type crystalline structure, with the value of K ranging between 2.8 and 4.0.

14 Claims, 9 Drawing Figures

FIG. 1 PRIOR ART



FIG. 2



FIG. 3



FIG. 4





FIG. 5

FIG. 6  
PRIOR ART

FIG. 7



FIG. 8



FIG. 9



## SUPERCONDUCTING MATERIALS

## BACKGROUND OF THE INVENTION

## 1. Field of the Invention

This invention relates to useful and novel superconducting materials and, more particularly, to improved intermetallic compound superconducting materials having high critical temperature and a  $\beta$ -W type crystalline structure generally represented by a formula  $(Nb_{1-y}Ta_y)_K (Al_{1-x}M_x)$ .

## BRIEF DESCRIPTION OF THE PRIOR ART

Many intermetallic compounds containing transition elements are found to have the  $\beta$ -W type crystalline structure. Many of these compounds have a superconducting character of high critical temperature  $T_c$ . Since the discovery of  $Nb_3Sn$  with a critical temperature of 18°K, about 63 different binary superconducting compounds have been found to date. Also, it has been found that there are many ternary and quaternary  $\beta$ -W type superconducting compounds having higher critical temperatures and high upper critical fields.

These type of compounds having the above excellent characters are thought to be very suitable as the material for superconducting magnet coils and superconducting transmission cables. However, the critical temperature  $T_c$  of  $\beta$ -W type binary compounds is only as high as 18°K in case of  $Nb_3Sn$  and  $Nb_3Al$ , and no superconductivity at higher temperatures has heretofore been obtained in binary compounds.

## SUMMARY OF THE INVENTION

An object of the invention is to provide a novel superconducting material, which has high critical temperature and can be readily manufactured as practical material, and with which it is possible to alleviate the cooling conditions in its practical use.

To achieve the above-noted object of the invention, part of Al in the  $Nb_KAl$  type structure is replaced with another element M, and also part of Nb is, if necessary, replaced with Ta. The value of K is set within a range from about 2.8 to about 4.0. The element substituted for Al and the quantity of partial substitution may be about 3.2 atomic percent or less of Pb or Ce, about 3.8 atomic percent or less of Bi or Te, about 4.4 atomic percent or less of Tl, about 6.4 atomic percent or less of Cu, about 5.8 atomic percent or less of Sb, about 4.2 atomic percent or less of Y, about 2.7 atomic percent or less of Pr or Eu, about 2.1 atomic percent or less of Ca, or about 7.2 atomic percent or less of Zn.

It is also effective, if necessary, to replace part of Nb with 4.0 atomic (at) percent or less of Ta. By substituting one of the aforementioned substitution elements for part of Al and if necessary Ta for part of Nb in the  $Nb_KAl$  type structure, it is possible to obtain compound superconducting materials having higher critical temperatures compared to the critical temperature (about 18°K at the highest) of the usual  $\beta$ -W type binary superconducting compounds such as  $Nb_3Al$ . According to the invention, it is possible to obtain critical temperatures higher than 19.3°K.

The invention is achieved as a result of detailed study and development of a McMillan's theoretical treatment on strong-coupled superconductors (W.L. McMillan; Phys. Rev. 167 (1968), p. 331), and is based on the finding that it is possible to obtain an increased superconducting critical temperature  $T_c$  by converting a su-

perconducting compound into a multi-element alloy in such a manner as to increase the averaged frequency  $\langle w \rangle$  of the phonon and the coefficient of electronic specific heat  $\mu$ .

## BRIEF DESCRIPTION OF THE DRAWINGS

FIG. 1 is a graph showing relations among critical temperature, averaged phonon frequency, pseudo-coulomb potential and electron-phonon coupling constant for some superconducting materials.

FIG. 2 shows relations between calculated value and observed value of Deby's temperature for some  $\beta$ -W type compounds.

FIG. 3 is a graph showing relations between electron-phonon coupling constant and coefficient of electronic specific heat for some  $\beta$ -W type compounds.

FIG. 4 is a graph showing relations between coefficient of electronic specific heat of some  $\beta$ -W type compounds and number of electrons per atom in the crystal.

FIG. 5 shows a model of C-D binary phase diagram with a showing of Deby's temperature and coefficient of electronic specific heat for  $Nb_3C_{1-x}D_x$  compounds plotted against x.

FIG. 6 shows four main types of binary diagram having an eutectic or eutectoid point.

FIG. 7 is a graph showing relations between critical temperature and concentration of element M for  $Nb_3(Al, M)$  alloys according to the invention.

FIG. 8 is a graph showing relations between critical temperature and concentration of Cu for  $(Nb, Ta)_3(Al, Cu)$  alloys according to the invention, with various concentrations of Ta.

FIG. 9 is a graph showing relations among critical temperature, K and x for  $Nb_K(Al_{1-x}Zn_x)$  alloys according to the invention.

## DETAILED DESCRIPTION OF THE INVENTION

The  $\beta$ -W type intermetallic compound  $Nb_3Al$  dealt with in the present invention is featured by a composite crystalline structure consisting of a body-centered cubic lattice formed by Al atoms, and Nb atoms lying in three perpendicular planes of the lattice. In this type of compound it is known that the critical temperature  $T_c$  is higher the closer the composition ratio thereof is to the stoichiometric one. Also, it is known that Nb-Nb atom chain in the  $\beta$ -W crystalline structure forms a very narrow d-band in the vicinity of the Fermi-level, thus increasing the Fermi-level d-electron state density and the superconducting critical temperature.

According to the McMillan's treatment (W.L. McMillan; Phys. Rev. 167(1968)331) on strong-coupled superconductors characterized by strong coupling between phonon and electron, the critical temperature  $T_c$  of a superconducting material is given as

$$T_c = \frac{\langle w \rangle}{1.45} \exp \frac{-1.04(1 + \lambda)}{\lambda - \mu^*(1 + 0.62)} \quad (1)$$

where  $\langle w \rangle$  is the averaged frequency of the phonon,  $\mu^*$  is the interelectron pseudo-coulomb potential, and  $\lambda$  is the electronphonon coupling constant. FIG. 1 shows the relationship among  $T_c/\langle w \rangle$ ,  $\lambda$ , and  $\mu^*$ . As is shown, the value of  $T_c/\langle w \rangle$  is greater the smaller is the value of  $\mu^*$  and the greater is the value of  $\lambda$ . Also,  $T_c$  is higher the greater is the value of  $\langle w \rangle$ .

The averaged phonon frequency  $\langle \omega \rangle$  is generally determined by the phonon spectrum, and in case of the  $\beta$ -W type structure it is approximately 1.3 times the Deby's temperature  $\theta_D$ . The value of  $\theta_D$  may be calculated from Lindemann's formula of melting point that holds well for simple metallic substances and alloys. In case of the  $\beta$ -W type crystalline structure, it is represented as

$$\theta_D = \frac{831.4}{a_0} \sqrt{\frac{T_m}{M_1}} \quad (2)$$

where  $a_0$  is the  $\beta$ -W type crystal lattice constant,  $T_m$  is the melting temperature, and  $M_1$  is the mean atomic weight.

FIG. 2 shows the correlation between observed Deby's temperature and calculated Deby's temperature for some known  $\beta$ -W type compounds. It will be seen that equation 2 holds fairly well although there is a tendency of forming clusters in dependence upon whether 3-d or 4-d band is occupied by the electrons of the element occupying the A site of intermetallic compounds represented by a general formula  $A_3C$ . Thus, it will be understood that to increase the value of  $\theta_D$  the compound should be converted into a multi-element material of a reduced lattice constant, an increased melting point and an increased molecular weight.

The value of  $\mu^*$  in equation (1) may be derived from the pseudo-coulomb potential theory, and in case of the  $\beta$ -W type structure it can be approximated by a constant of  $\mu^*=0.13$ .

The third parameter  $\lambda$  can be defined by the McMillan's theory as mentioned earlier. It may also be obtained semiexperimentally from known data as shown in FIG. 3, in which the electron-phonon coupling constant and coefficient of electronic specific heat  $\gamma$  are correlated for known  $\beta$ -W type compounds. As is shown, the relation between  $\gamma/\lambda$  and  $\gamma$  is represented by a straight line, whose x - or y-intercept differs in dependence upon the d-band that is occupied by the electrons of the element occupying the A site of the compound  $A_3C$  but whose slope is the same in either case. In this way, there holds a linear relation between  $\gamma$  and  $\lambda$  for a group of compounds having the same d-band structure. Thus, the value of  $\lambda$  may be determined if the magnitude of  $\gamma$  is determined. The parameter  $\gamma$  may also be obtained from data as shown in FIG. 4, in which  $\gamma$  of various  $\beta$ -W type compounds  $A_3C$  is plotted against the number  $Z$  of electrons per atom in the  $\beta$ -W type crystal, that is, the ratio between total electron number  $e$  and atom number  $a$ . In this case, the value of  $\gamma$  greatly varies in dependence upon which of 3-d, 4-d and 5-d bands is occupied by the electrons of the high melting transition element occupying the A site. Also, it will be seen that the value of  $\gamma$  continuously changes with  $Z$  depending upon the kind of element occupying the C site.

In accordance with the invention, in order to increase the critical temperature  $T_c$ , either the A site or the C site of the  $\beta$ -W type binary superconducting compound  $A_3C$  is partially replaced with a suitable different element or both sites are replaced with suitable different elements to obtain multi-element superconducting compounds having  $T_c$  higher than that of the mother material.

The  $\beta$ -W type multi-element superconducting compounds obtained by incorporating two different foreign metals are generally represented as



The critical temperature of this type of material is greatly influenced not only by the kind of the substitution elements B and D but also by the composition ratios ( $x, y$  and  $K$ ) and various heat treatment conditions.

10 Taking  $Nb_K(C_{1-x}D_x)$  as an example of the multi-element compounds, to make  $T_c$  highest by selecting composition it is necessary to select  $K$  to be coincident with the stoichiometrical ratio, and best results may be obtained if it is in a range  $2.8 \leq K \leq 4.0$ .

15 If the value of  $K$  is less than 2.8, the superconducting character would be deteriorated due to generation of such compounds as  $Nb_2(C, D)$ . The critical temperature  $T_c$  will be the highest with a value of  $K$  in the proximity of 3.0. With this value of  $K$ , however, the range 20 of  $x$  with which it is possible to expect satisfactory results is very narrow. With greater values of  $K$  the critical temperature  $T_c$  may be increased for a broader range of  $X$ , but the highest value of  $T_c$  would be reduced. If the value of  $K$  exceeds 4.0, the superconducting character will be deteriorated.

25 In another aspect, the concentration  $x$  of the element D should be selected to be in the proximity of the composition corresponding to the eutectic point of a binary eutectic alloy of C and D. The upper half of FIG. 5 is 30 a model of C-D binary phase diagram, and the lower half of FIG. 5 shows the Deby's temperature and coefficient of electronic specific heat for  $Nb_3C_{1-x}D_x$  compounds plotted against  $x$  corresponding with the upper half. It will be seen from this FIGURE that the Deby's 35 temperature of the  $Nb_K(C, D)$  compound is the highest and the coefficient of electronic specific heat is large for the composition corresponding to the eutectic point of the elements occupying the C site. Accordingly, by 40 selecting the concentration  $x$  of the element D in the system given as  $Nb_K(C_{1-x}D_x)$  to be in the proximity of a value for the composition corresponding to the eutectic point of the C-D alloy, the superconducting character of  $Nb_KC$  compound may be improved particularly 45 at the critical temperature thereof.

FIG. 6 shows four main types of phase diagrams of C and D, corresponding to  $A_3C$  and  $A_3D$  combinations, the D component occupying the C site in case of having Nb as the element A and Al as the element C. Namely, 50 there are Pb type, Cu type, Sb type with some varieties and eutectoid type. Of these combinations, those which can meet conditions for rendering into multi-element material having high  $T_c$  are  $Nb_3(Al-Pb)$ ,  $Nb_3(Al-Bi)$  and  $Nb_3(Al-Tl)$  as the Pb type,  $Nb_3(Al-Cu)$  as the Cu type,  $Nb_3(Al-Sb)$ ,  $Nb_3(Al-Te)$ ,  $Nb_3(Al-Y)$ ,  $Nb_3(Al-Ce)$ ,  $Nb_3(Al-Pr)$ ,  $Nb_3(Al-Eu)$  and  $Nb_3(Al-Ca)$  as the Sb type and  $Nb_3(Al-Zn)$  as the eutectoid type. In any of these materials the critical temperature  $T_c$  is higher compared to  $Nb_3Al$ .

55 For each of these combinations the aforementioned effective composition range applies. A concentration of the element D higher than the above range is undesired because reduction of  $T_c$  results.

60 It is to be noted that satisfactory results may be obtained not only with alloys where part of Al of the superconducting alloy represented as  $Nb_KAl$  is replaced with one of the aforementioned substitution elements,

but also by replacing part of Al with two or more members of the group of the aforementioned elements.

An additional effect of increasing the critical temperature  $T_c$  may be obtained by incorporating Ta, which takes a coordination number of 12 and whose atomic radius is slightly smaller than that of Nb. In this case, the desired concentration  $x$  of the element D corresponding to the proximity of the eutectic point of the C-D alloy tends to be slightly influenced by the concentration  $y$  of the element Ta, but the resultant deviation may be empirically determined.

#### DESCRIPTION OF THE PRESENTLY PREFERRED EMBODIMENTS

The following examples are given in order for the invention to be more fully understood.

##### EXAMPLE 1

This example deals with  $\beta$ -W type ternary superconducting materials represented by a formula  $Nb_3Al_{1-x}M_x$  where M is a member of a group consisting of Pb, Bi, Tl, Cu, Sb, Te, Y, Ce, Pr, Eu, Ca and Zn.

Samples of materials with compositions containing the above elements were obtained through a combination of plasma arc melting or sintering and levitation melting. Materials in the form of masses and with purities of at least 99.99 percent are weighed to prepare predetermined compositions, and the resultant compositions were subjected to plasma arc melting in an argon atmosphere under pressure of around 1 atm. to produce button-like masses. These button-like masses were inverted several times for sufficient alloying. To obtain samples having a shape convenient for the measurement of  $T_c$ , the button-like masses were subjected to levitation melting in an argon atmosphere, and the resultant fused materials were cast into water-cooled copper molds to produce rod-like samples. In case of combinations including an element having sufficiently low melting point and vapor pressure compared to the high-melting transition element Nb, (for instance where M is Ca, Zn, Sb, Te, Ce, Pb or Tl), powdery materials were used, and predetermined compositions were sufficiently mixed and press molded with a pressure of 1 ton/cm<sup>2</sup>. The resultant moldings were temporarily sintered in an argon atmosphere under a pressure of about 1.5 atm. and at a temperature of not higher than 1,000°C. to produce samples containing low-grade intermetallic compounds poor in Nb, which were then subjected to levitation melting as mentioned above to produce rod-like samples.

Many of the samples obtained in the above manner had a diameter of 3 mm and a length of 30 mm, but some samples were too brittle to have the length of 30 mm. These cast samples were wrapped with a Nb foil and sealed within a quartz ampoule evacuated to a vacuum degree of  $10^{-6}$  Torr. for heat treatment at a predetermined temperature within a range between 600° and

1,200°C. for 1 to 15 days followed by sudden cooling with water and thus became aged materials. The stoichiometrical composition ratio K and atomic concentration x of the resultant samples were examined by chemical quantitative analysis, and the weight reduction of various components after the melting was within a range of several percent. Also, many of these samples were so brittle that they can be sufficiently crushed to study their crystal structure by the Deby's X-ray refraction method. By this analysis it was found that the superconducting materials according to the invention with Al in the  $Nb_3Al$  partially replaced with the substitution element M showed typical refraction pattern of the  $\beta$ -W type crystalline structure for a range of  $x$  up to nearly  $x = 0.25$  in case where M is Ca, Te, Ce, Pr, Eu or Tl and for a range of  $x$  up to nearly 0.5 in case where M is Cu, Zn, Sb, Y, Pb or Bi.

The critical temperature  $T_c$  of the samples obtained in the above manner was measured by the usual four resistance probe technique. More particularly, the critical temperature  $T_c$  is set to the temperature when the resistance recovered and just reaches one half of the difference of resistance between the superconducting state and normal state, wherein the sample is 30 mm long carries a constant current of several amperes per square centimeter between its ends.

FIG. 7 shows relations between critical temperature  $T_c$  and atomic concentration or atomic percent  $x$  of the element M for various  $Nb_3Al_{1-x}M_x$  ternary alloys having been subjected to a heat treatment at a temperature of 700°C. for 100 hours. Where M is Pb, Ce, Bi, Te, Pr, Eu or Ca, the critical temperature  $T_c$  is the highest when about 1.25 atomic percent of Al is replaced with the third element M, that is, when x is set to about 0.05. The eutectic point of these Al-M systems lies between 1 and 5 atomic percent of the concentration of the element M, which substantially corresponds to the value of  $x$  of the element M when the critical temperature  $T_c$  is at its peak. Where M is Zn, Cu, Sb, Y or Tl, the critical temperature  $T_c$  is relatively high when up to about 5.0 atomic percent of Al is replaced with the element M, that is, for values of  $x$  up to about 0.2, and the concentration  $x$  of the element M corresponding to the peak of the critical temperature  $T_c$  substantially coincides with the corresponding concentration at the eutectic point of the Al-M system except for the case where M is Sb. The highest critical temperature obtained was 19.3°K with  $Nb_3(Al, Zn)$ .

From FIG. 7, Table 1 below lists the concentration range of the element M necessary to obtain  $T_c$  higher than about 18°K, the concentration range of the element M necessary to obtain  $T_c$  higher than about 18.5°K and the most desirable concentration range of the element M to increase  $T_c$ . The presence of about 0.05 atomic percent of M except for Sb leads to appreciable effects, while the presence of about 2 atomic percent of Sb leads to appreciable effects.

Table 1

| Element M | Concentration range of M (in atomic %) for $T_c > 18^{\circ}\text{K}$ | Concentration range of M (in atomic %) for $T_c > 18.5^{\circ}\text{K}$ | Most desired concentration range of M (in atomic %) |
|-----------|-----------------------------------------------------------------------|-------------------------------------------------------------------------|-----------------------------------------------------|
| Pb, Ce    | <3.2                                                                  | 0.2 - 2.8                                                               | 0.9 - 1.6                                           |
| Bi, Te    | <3.8                                                                  | 0.2 - 3.2                                                               | 0.9 - 1.6                                           |
| Tl        | <4.4                                                                  | 0.2 - 3.9                                                               | 0.9 - 1.6                                           |
| Cu        | <6.4                                                                  | 0.6 - 5.3                                                               | 2.1 - 2.9                                           |

Table 1 - Continued

| Element M | Concentration range of M (in atomic %) for $T_c > 18^{\circ}\text{K}$ | Concentration range of M (in atomic %) for $T_c > 18.5^{\circ}\text{K}$ | Most desired concentration range of M (in atomic %) |
|-----------|-----------------------------------------------------------------------|-------------------------------------------------------------------------|-----------------------------------------------------|
| Sb        | <5.8                                                                  | —                                                                       | 4.6 - 5.4                                           |
| Y         | <2.4, 3.2 - 4.2                                                       | 0.6 - 1.9                                                               | 0.9 - 1.6                                           |
| Pr, Eu    | <2.7                                                                  | 0.3 - 2.3                                                               | 0.9 - 1.6                                           |
| Ca        | <2.1                                                                  | 0.3 - 1.9                                                               | 0.9 - 1.6                                           |
| Zn        | <7.2                                                                  | 0.2 - 5.8                                                               | 0.9 - 1.6                                           |

## EXAMPLE 2

This example deals with quarternary superconducting materials obtained by replacing part of Nb with Ta in the samples in the first example.

FIG. 8 shows relations between critical temperature  $T_c$  and concentration for Cu for  $\beta$ -W type intermetallic compounds according to the invention having compositions of  $(\text{Nb}_{0.98}\text{Ta}_{0.02})_3(\text{Al}_{1-x}\text{Cu}_x)$ ,  $(\text{Nb}_{0.95}\text{Ta}_{0.05})_3(\text{Al}_{1-x}\text{Cu}_x)$  and  $\text{Nb}_3(\text{Al}_{2-x}\text{Cu}_x)$ . The samples in this embodiment were prepared as in Example 1.

It will be seen that the critical temperature of materials obtained by replacing part of Nb with Ta in the  $\text{Nb}_3(\text{Al},\text{M})$  system is higher, although slightly, compared to that of samples without incorporating Ta. The range of concentration of Ta to obtain the above effects is less than about 4.0 atomic percent.

## EXAMPLE 3

This example deals with ternary superconducting materials obtained by changing the concentration of Nb in the samples in the first example.

FIG. 9 shows relations between critical temperature  $T_c$  and concentration of Zn for alloys having  $\beta$ -W type crystalline structure and composition of  $\text{Nb}_K(\text{Al}_{1-x}\text{Zn}_x)$  when K is 2.8, 3.0 and 4.0 respectively. The method of preparation of samples and method of measurement of the critical temperature are similar to the previous first and second examples.

This example reveals that alloys represented as  $\text{Nb}_K(\text{Al}_{1-x}\text{M}_x)$  show high critical temperatures when K is within a range of  $2.8 \leq K \leq 4.0$ . If the value of K is smaller than 2.8, no appreciable improvement of the critical temperature can be obtained. Also, where x representing the concentration of the element M substituted for Al is less than about 0.15, the critical temperature is highest with a value of K in the proximity of 3.0. For greater values of x, better results may be obtained with values of K greater than 3.0. However, with values of K greater than 4.0 the characteristics of the material becomes instable, and satisfactory results cannot be expected.

Similar results with respect to the value of K were obtained where M is other elements than Zn. The concentration of Nb corresponding to the above range of K is about 74 to 80 atomic percent. As has been mentioned in the second embodiment, less than about 4 percent of Nb may be replaced with Ta, and in such case the lower limit of the concentration of Nb is about 70 atomic percent.

As has been described above in detail, the superconducting materials according to the invention, said materials having  $\beta$ -W type crystalline structure and, multi-element compounds which have novel composition of  $\text{Nb}-\text{Al}-\text{M}$  or  $\text{Nb}-\text{Ta}-\text{Al}-\text{M}$  (where M is a member selected from the group consisting of Pb, Bi, Tl, Cu, Sb, Te, Y, Ce, Pr, Eu, Ca and Zn) have higher critical tem-

perature  $T_c$  ( $19.3^{\circ}\text{K}$  at the highest) compared to that of the  $\text{Nb}_3\text{Al}$  materials and have characteristics sufficient for use as practical material.

15 What is claimed is:

1. A superconducting material having high critical temperature, said material being an alloy represented by the formula:  $\text{Nb}-\text{Al}-\text{M}$ , wherein M is an element selected from the group consisting of 0.05-3.8 atomic percent of Te, 0.05-2.4 atomic percent of Y, 3.2-4.2 atomic percent of Y, 0.05-3.2 atomic percent of Ce, 0.05-2.7 atomic percent of Pr, 0.05-2.7 atomic percent of Eu, 0.05-2.1 atomic percent of Ca and 0.05-7.2 atomic percent of Zn, wherein the amount of Nb is in a range of 74-80 atomic percent and the balance of said alloy is Al and very minor amounts of unavoidable impurities.

2. The superconducting material of claim 1, in which less than 4 percent of Nb is replaced with an equal amount of Ta.

3. The superconducting material of claim 1, in which M is 0.05-3.8 atomic percent of Te.

4. The superconducting material of claim 1, in which M is 0.05-2.4 atomic percent of Y.

5. The superconducting material of claim 1, in which M is 3.2-4.2 atomic percent of Y.

6. The superconducting material of claim 1, in which M is 0.05-3.2 atomic percent of Ce.

7. The superconducting material of claim 1, in which M is 0.05-2.7 atomic percent of Pr.

8. The superconducting material of claim 1, in which M is 0.05-2.7 atomic percent of Eu.

9. The superconducting material of claim 1, in which M is 0.05-2.1 atomic percent sign of Ca.

10. The superconducting material of claim 1, in which M is 0.05-7.2 atomic percent of Zn.

11. A superconducting material having high critical temperature greater than  $18.5^{\circ}\text{K}$ , said material being an alloy represented by the formula  $\text{Nb}-\text{Al}-\text{M}$ , where M is an element selected from the group consisting of 0.2-3.2 at percent of Te, 0.6-1.9 at percent of Y, 0.2-2.8 at percent of Ce, 0.3-2.3 at percent of Pr, 0.3-2.3 at percent of Eu, 0.3-1.9 at percent of Ca and 0.2-5.8 at percent of Zn, wherein the amount of Nb is in a range of 74-80 percent and the balance of said alloy is Al and very minor amounts of unavoidable impurities.

12. The superconducting material of claim 11, in which less than 4 percent of Nb is replaced with an equal amount of Ta.

13. The superconducting material of claim 11, in which said M is an element selected from the group consisting of 0.9-1.6 at percent of Te, 0.9-1.6 at percent of Y, 0.9-1.6 at percent of Ce, 0.9-1.6 at percent of Pr, 0.9-1.6 at percent of Eu, 0.9-1.6 at percent of Ca and 0.9-1.6 at percent of Zn.

14. A superconducting material having high critical temperature, said material being represented by a formula  $(Nb_{1-y}Ta_y)_K (Al_{1-x}M_x)$ , wherein M is an element selected from the group consisting of Te, Y, Ce, Pr, Eu, Ca and Zn, and wherein the value of y and K are  $y \leq$

0.05 and  $2.8 \leq K \leq 4.0$  respectively, and the value of x approximately corresponds to the value of Z in an eutectic alloy represented by a formula  $Al_{1-z}M_z$ .

\* \* \* \* \*